

## UNITED STATES PATENT OFFICE.

HERMAN M. CASTNER, OF NOBLEBORO, MAINE.

## PROCESS OF MAKING COMPRESSED FIBER BOARD.

No Drawing.

Application filed August 8, 1921. Serial No. 490,759.

*To all whom it may concern:*

Be it known that I, HERMAN M. CASTNER, a citizen of the United States, and resident of Nobleboro, in the county of Lincoln and 5 State of Maine, have invented certain new and useful Improvements in Processes of Making Compressed Fiber Board, of which the following is a specification.

My present invention relates to an improved 10 product or article of manufacture which I term "Ivory fiber board" and to the process of making the same.

The invention aims to produce a product which may be used as a leather substitute 15 in the manufacture of white shoes, though not limited to this use, and which will be flexible and elastic and free from all danger of splitting or cracking.

The invention further aims to provide a 20 product which may be built up into a number of layers or laminations which will be permanently united and free from all danger of separating.

A further object is to secure a product 25 which will retain its original color appearance for an indefinite period.

With these and other objects in view, the invention includes the novel product and process hereinafter described and particularly defined by the appended claims.

In proceeding according to my improved process I take bleached white sulphite wood pulp of the best quality, to which is added about ten per cent of paraffin paper or any 35 form of paraffin waste. This is mixed with water and beat into a pulp by a power beater for the period of an hour or more, depending upon the condition of the material. From there it passes into an agitator tank where fifty per cent of water is 40 added and the whole thoroughly mixed. It is further put through two centrifugal pumps to get it properly mixed and of the right consistency, passing by means of the 45 pumps into a tank which supplies the material for what is known as a wet machine. This is the machine on which the board is made as later described.

At this point one hundred per cent of 50 water is added and the whole mixture is then picked up by a wire-covered cylinder, passed on to a felt and press roll until roll has accumulated thereon a substance of

proper thickness, when it is cut off, taken from roll and next passed to the dry room. 55

Three tons of the board as taken from the cylinder produces about one ton of finished product after it has been dried and tempered. In the dry room it is placed upon racks made of wire screening, one sheet 60 upon a rack, these racks being about an inch apart, and dried in a moist atmosphere, which prevents the material from becoming hard and brittle so that it will split in the nailing, or in other words, makes it flexible and elastic. If the board is too soft, it 65 will separate into layers, and if it is too hard it will split in the nailing, but the moist air in drying is what makes it tough, flexible and of the right consistency. 70

The board is finished by being run through hydraulic rolls under several tons pressure. When finished it is dry, but tough, flexible and elastic.

The mixture of material makes a fast 75 ivory color which will not change except as the ivory takes a somewhat deeper shade by age.

The drying is preferably done by steam in a large room well ventilated, with fans 80 to keep up a circulation of air. It is dried evenly, so that the finished board will not curl up.

I claim:

1. The herein described method which consists in commingling sulphite wood pulp with approximately ten per cent of paraffin and water, thereafter adding additional water to the mass and thoroughly agitating the same, adding further water, and then forming the mixture into sheets, drying the sheets in a moist atmosphere, and subjecting the sheets to pressure. 85

2. The herein described method which consists in mixing bleached white sulphite wood pulp with approximately ten per cent of paraffin in the presence of water, thoroughly agitating the mixture in the presence of additional water, forming the mixture into layers, drying said layers in a moist 90 atmosphere, and subjecting the same to pressure. 95

In testimony whereof, I affix my signature.

HERMAN M. CASTNER.